

May 25, 1954

R. D. HALL

2,679,569

ELECTRICALLY CONDUCTIVE FILM

Filed Aug. 25, 1951

*Fig. 1.*



*Fig. 2.*



*Fig. 3.*



*Fig. 4.*



RALPH D. HALL,  
INVENTOR.

BY *Horatio White*

ATTORNEY.

## UNITED STATES PATENT OFFICE

2,679,569

## ELECTRICALLY CONDUCTIVE FILM

Ralph D. Hall, Pacoima, Calif., assignor to Electrofilm Corporation, Los Angeles, Calif., a corporation of California

Application August 25, 1951, Serial No. 243,733

10 Claims. (Cl. 201—73)

1

This invention relates to improved electrical resistor elements of a type comprising a thin electrically conductive film or coating applied to the surface of a base or carrier member. Conductive films formed in accordance with the invention are adapted for a wide variety of heating and electrical resistance uses, as for instance for heating the surface of an aircraft part to prevent its icing, or for radiating heat from a wall to which the film is applied to warm a room.

The resistor films of the present invention include an electrically insulative binder material, within which is distributed a preferably finely divided conductive material of a nature to give the composite film the desired resistance characteristics. In use, electricity is supplied to the film through a pair of electrodes or terminals electrically connected to the film at spaced locations.

A particular difficulty encountered in many prior films of the above general type has been their tendency to badly overheat or burn due to changes in their electrical resistances. One important object of the present invention is to provide a film so constituted as to prevent such excessive overheating or burning. This result may be achieved in large part by predetermination of the temperature coefficient of resistance of the film, and specifically by so forming the film that its coefficient has a positive value over the usable temperature range. When the film is given such a positive temperature coefficient, its resistance increases with a rise in temperature, so that the film itself acts to limit accumulative current increases, and prevent the cumulative heating which characterizes a negative coefficient. Best operating results have been achieved when the positive temperature coefficient is of a value below about +.004 per degree C.

For purposes of definiteness, the term "temperature coefficient of resistance," as used in this application, is defined as the value of  $\alpha_{ref}$  in the following formula:

$$R_t = R_{ref}(1 + \alpha_{ref}t)$$

where  $R_t$ —resistance at  $t^{\circ}\text{C}$

$R_{ref}$ —Original resistance at a (different) reference temperature, and

$\alpha_{ref}$ —T. C. R. at the reference temperature (for instance 0° C.)

To attain a composite film having both a predetermined resistance value and a predetermined temperature coefficient, two or more different conductive materials are distributed through the

5 binder in proportions to produce the desired characteristics. In accordance with the invention, one of these conductive materials is a metal, normally having a positive coefficient, while a second of the materials may have a lower or negative coefficient partially counteracting the positive coefficient of the metal. As the metal, I may typically use elemental silver, nickel, or zinc, or a metallic alloy, such as stainless steel. For best 10 results, the second material should be carbon, preferably in the form of finely divided graphite having a negative coefficient.

In many instances, it has been found that incorporation of only the above materials in a 15 binder cannot produce a film of a particular resistance without at the same time giving to the film a negative temperature coefficient. For this reason, I often find it desirable to distribute within the binder an additional resistance material adapted to increase the resistance of the composite film while maintaining its positive coefficient. This third material may be characterized broadly as having a greater resistance than the composite film, and usually itself has a negative coefficient, though not of a value to give a negative coefficient to the film. Good results have been achieved by using as the resistance material a metallic oxide, such as antimony oxide, titanium dioxide, zinc oxide, chromic oxide or ferric oxide. Of the various oxides, antimony oxide and titanium dioxide have proven most desirable for the purpose.

Great difficulty has been encountered in previously proposed films of the present type by reason of their very unpredictable, unstable, and non-uniform characteristics. Different films made of exactly the same constituents in exactly the same proportions, but varying in the physical relation of the components, have often had widely differing electrical resistances, and as a result it has generally been considered impossible to accurately predetermine the resistance of a film. In accordance with the present invention, I am able to overcome these disadvantages of prior expedients, and to produce elements whose resistance characteristics may be very closely predicted, so that an element may be predesigned for any desired use. This predeterminability of the film resistance, and an accompanying uniformity and stability of resistance characteristics, are all achieved in large part by special formation of the various conductive and resistance particles in the film. For this purpose, it has been found desirable that the particles of either the metal or carbon, and preferably both,

be in flake form. As will be appreciated, such flake formation of these materials maximizes the likelihood that each individual particle will form an effective electrical contact with adjacent particles, to provide a uniform and continuous electrical circuit across the entire extent of the film. In addition to improving the resistance characteristics of the film, the use of flaky particles serves to strengthen and integrate the film, by reason of the interfitting (i. e. overlapping or shingle-like) relationship of adjacent flakes, in a manner preventing cracking of the film and resultant breaking of the electrical circuit upon changes in film temperature.

The predeterminability and uniformity of film resistance has been further enhanced by forming the particles of some or all of the binder carried materials of such extremely small sizes as to cause their virtually completely uniform dispersion throughout the entire film. For this purpose, it is desirable that the carbon particles have maximum dimensions not greater than about 10 microns, and preferably between about 1 and 5 microns; and that the metal and metallic oxide particles have maximum dimensions not greater than about 40, and preferably less than about 15 microns.

Many of the insulative binder and some of the other materials used in the present films are of an inflammable nature, and it is consequently desirable to provide some means for preventing their burning. For this purpose, I may incorporate in the film composition a fire retardant material, preferably in finely divided uniformly distributed condition, of a type not chemically reactive with the other film constituents, and adapted to remain stable under normal operating conditions and temperatures, but to produce a flame quenching gas when heated to a temperature above about 600° F., as by burning of the binder. I may employ for this purpose a chlorinated hydrocarbon plasticizer, such as the chlorinated polyphenyl sold by Monsanto Chemical Co., of St. Louis, Mo., under the trade name Aroclor, adapted to release flame smothering chlorine gas when heated above 600° F. Other satisfactory fire retardants include the chlorinated hydrocarbons sold by Monsanto Plastics Co. of St. Louis, Mo., under the trade names Santisizer 141 and Santisizer 160. It is noted that when the metallic oxide is employed as the resistance material in the present films, it also serves to a certain extent as a fire retarding element for aiding in preventing burning of the film.

The nonconductive binder may be of any of various known materials adapted to withstand the particular conditions to which the film is to be subjected. Where the film is to be applied to a substantially rigid member, the binder may be a suitable resin, preferably a thermosetting alkyd, phenolic, furfural, vinyl, or silicon resin. If it is desired to apply the conductive film to a flexible member, such as a tape, the binder may be a suitable elastomer, such as Buna N, neoprene, natural rubber, or a silicone rubber. Best results have been attained by using between about 60 to 110 parts binder by weight to 100 parts by weight of the materials distributed within the binder. In order to prevent the binder from reacting chemically with the metal particles and oxidizing, it is desirable that the binder have a pH between about 6 and 8, or in other words be approximately neutral.

The film composition may be applied to a surface by spraying, knife spreading, or any other

convenient method. Ordinarily, the composition is first thinned to a spraying or spreading consistency by the addition of a suitable solvent. For this purpose, I may employ any of the conventional solvents for the particular binder being used, as for instance a hydrocarbon, alcohol, ketone, ester or ether solvent. After application, the composition is heated to a temperature sufficient to drive off the solvent and cure the resin or other binder. The conductive film exhibits best operating characteristics when of a thickness between about .001" and .025", and is preferably about .006". A film less than .001" thick has a less uniform electrical resistance than a film within the defined range, and when the thickness is greater than .025", the likelihood of the film's cracking and thus breaking the electrical circuit increases. However, the unit resistance (ohm/sq.) is governed by the constituents and not the element thickness.

As a first example of the present invention, a very stable and uniform resistance film has been formed from the following constituents, mixed in the designated proportions by weight: 27.5 parts amorphous graphite, maximum particle dimension 10 microns, purchased from Joseph Dixon & Co., Jersey City, N. J., under the manufacturer's number 200-18; 27.5 parts antimony oxide; 45 parts flake silver, maximum flake dimension 40 microns, sold by Metals Disintegrating Company, Elizabeth, New Jersey, under the product No. MD585; 8 parts fire retardant chlorinated hydrocarbon plasticizer, sold by Monsanto Chemical Company, St. Louis, Mo., under the trade name Aroclor 1254; and 80 parts alkyd resin. These ingredients were intimately mixed together and thinned to spraying consistency with Xylene solvent, after which they were sprayed onto an insulating base film of the alkyd resin. A conductive film of the above composition .006" thick had a uniform electrical resistance of approximately 3 ohms per square. In this connection, it is noted that where the term "ohms per square" is used in this application, I refer to the resistance of a square element of any size, the resistance being the same regardless of the dimensions of the square. The individual temperature coefficients of resistance of the silver and graphite particles used in the above example were +.006 and -.004 per degree C. respectively, and the coefficient of the composite film was +.00098 per degree C.

In a second example of the invention, the above constituents were mixed in the following proportions by weight: 30 parts amorphous graphite; 30 parts antimony oxide; 40 parts silver; 8 parts Aroclor 1254; and 80 parts resin.

A third typical formula was of the following composition, proportions again being taken by weight: 11.5 parts nickel flake, maximum flake dimension 40 microns, sold by Metals Disintegrating Company, Elizabeth, New Jersey, under the product No. MD750; 68.6 parts "Merrillite" zinc precipitate, maximum particle size 40 microns, sold by Alloys Division Metals Disintegrating Company, Berkeley, California; 10 parts amorphous graphite, maximum particle dimension 10 microns; 80 parts alkyd resin; and 4 parts Aroclor 1254. The electrical resistance of a .006" film of this last composition was approximately 12 ohms per square. The temperature coefficients of resistance of the nickel, zinc and graphite were +.0003, +.005 and -.004 per degree C. respectively, and the coefficient of the composite film was +.00013/° C.

Where the aircraft part, wall or other member carrying a conductive film of the present invention is itself of an electrically conductive nature, an insulative layer may be applied to the member before application of the conductive film. Certain particular features of the invention have to do with improved means for assuring an adequate and continuous bond between such an insulative base layer and the resistance film. Specifically, the effectiveness of the bond may be maximized by (1) forming the base layer and conductive film to have approximately equal coefficients of expansion, and (2) applying the films in a manner such that some of the particles in the conductive film diffuse into the insulative film, to reinforce the inter-layer bond. This last feature of the invention and certain others, will be better understood from the following detailed description of the typical embodiments illustrated in the accompanying drawing, in which:

Fig. 1 is a fragmentary perspective view of a heating or resistance film embodying the invention and shown applied to a rigid base member;

Fig. 2 is an enlarged fragmentary sectional view taken on line 2—2 of Fig. 1;

Fig. 3 is an enlarged fragmentary sectional view on the scale of Fig. 2, and showing a preferred method for reducing the thickness of the applied film to a desired and uniform dimension; and

Fig. 4 shows a flexible film applied to a flexible woven fabric.

Referring first to Figs. 1 and 2, I have typically represented at 10 a rigid base member to which an insulating film 11 and the heating or resistance film 12 are applied. The base member may be any member whose surface is to be heated, or across whose surface electricity is to be conducted, as for instance an aircraft part to be maintained against icing, or the wall of a room to be heated.

The electrically insulative base layer or film 11 is first applied to the surface of the member 10, and then separately thermally cured. The insulative layer may typically comprise an electrically non-conductive binder material containing high dielectric particles, such as mica or vermiculite, distributed throughout the binder. The binder of film 11 may be any of the binders listed above as usable in the conductive film 12, and in order to assure a permanent bond between films 11 and 12, is preferably so chosen as to give the two films approximately the same coefficient of expansion. In many instances, the same binder is used for both films. A typical formula for the insulative film includes 60% binder, 20% mica and 20% vermiculite.

After the insulative layer 11 has been applied and cured, the conductive film 12 is sprayed onto, or otherwise applied to, the outer surface of layer 11. The binder in the conductive film is then thermally cured, to simultaneously integrate the constituents of the film, and bond it to the base layer. The heat of curing the binder in conductive film 12 softens insulative layer 11 to an extent such that some of the particles 13 migrate downwardly into an upper portion of layer 11 at 14, to positively assure a tight mechanical bond between the two films.

For passing electrically through the film, a pair of elongated electrodes 15 and 16 may be fastened to the surface of the conductive film at a pair of spaced locations. These electrodes may be attached to the film in any suitable manner, as by bolts 17 passing upwardly through member

10 and the two films. The upper ends of bolts 17 may serve as the terminals to which current supply cables 18 are connected.

Spraying and other conventional application methods sometimes do not produce films of sufficiently accurate and uniform thickness to assure predetermined resistance characteristics. Consequently, after the uncured composition for one of the films has been applied, it is sometimes desirable to smooth the film to a desired thickness in the manner represented in Fig. 3. Specifically, an elongated knife 19 extending across the film may be moved along the upper side of the film in predetermined spaced relation to base member 10, to level off the entire film to a predetermined desired thickness.

Fig. 4 represents the manner in which a conductive film 20 embodying the invention may be applied to a flexible fabric or tape 21, instead of the rigid base member of Fig. 1. In order to permit flexure of the film with the tape, the film binder may be a suitable elastomer in this instance, such as Buna-N, neoprene, natural rubber, or a silicone rubber. The tape may have an adhesive material 22 at its side opposite the film 20, to facilitate application of the tape to a carrier surface.

I claim:

1. A heating element comprising a base material carrying a hardened and dimensionally stabilized thin electrically conductive film having resistive heating properties and comprising an initially fluid binder cured to permanently solid non-conductive form and containing uniformly distributed solid conductive flaky metal particles having relatively higher temperature coefficient of resistance admixed uniformly with resistive flaky graphite particles having lower temperature coefficient of resistance, said metal particles being predominantly under 40 microns in size and the graphite particles being predominantly under 10 microns in size, and said film resulting from curing a quantity of the binder with the flaky metal and graphite particles in interfitting relation therein sufficient to permanently so maintain the flakes in the binder.

2. A heating element as claimed in claim 1, in which the majority of said metal particles are under 15 microns in size.

3. A heating element as claimed in claim 1, in which said film has a positive temperature coefficient of resistance below about +0.004.

4. A heating element as claimed in claim 1, including finely divided metal oxide uniformly distributed within the film and having a lower coefficient of resistance than said metal particles.

5. A heating element as claimed in claim 1, including antimony oxide uniformly distributed within the film.

6. A heating element as claimed in claim 1, in which said metal particles are flake silver.

7. A heating element as defined in claim 1, in which said binder is a thermosetting resinous plastic material and said metal particles are elemental silver.

8. A heating element as claimed in claim 1, including a chlorinated hydrocarbon fire retardant uniformly distributed within the film.

9. A heating element as claimed in claim 1, in which said binder is a silicone rubber.

10. A heating element as claimed in claim 1, in which said metal particles are silver particles under 15 microns in size, said binder is a thermo-

setting resinous material, and said film contains a metallic oxide uniformly distributed therein.

References Cited in the file of this patent

UNITED STATES PATENTS

| Number    | Name         | Date          |
|-----------|--------------|---------------|
| 1,994,967 | Sklar        | Mar. 19, 1935 |
| 2,060,114 | Podolsky     | Nov. 10, 1936 |
| 2,247,036 | Ruben        | June 24, 1941 |
| 2,301,882 | Kappeler     | Nov. 10, 1942 |
| 2,437,708 | Plass et al. | Mar. 16, 1948 |
| 2,442,810 | Haas         | June 8, 1948  |
| 2,452,805 | Sussenbach   | Nov. 2, 1948  |
| 2,479,914 | Drugmand     | Aug. 23, 1949 |
| 2,494,920 | Warrick      | Jan. 17, 1950 |

| Number    | Name     | Date          |
|-----------|----------|---------------|
| 2,495,199 | Podolsky | June 17, 1950 |
| 2,530,217 | Bain     | Nov. 14, 1950 |

FOREIGN PATENTS

| Number  | Country       | Date          |
|---------|---------------|---------------|
| 153,380 | Great Britain | Feb. 7, 1921  |
| 490,232 | Great Britain | Aug. 11, 1938 |

OTHER REFERENCES

|    |                                                                                                                 |
|----|-----------------------------------------------------------------------------------------------------------------|
| 10 | Nat. Bureau of Std. Circular 468, Nov. 15, 1947, pp. 5-9.                                                       |
| 15 | Zimmerman & Lavine, "Handbook of Material Trade Names," Industrial Research Service, Dover, N. H., 1946, p. 46. |